

## UNITED STATES PATENT OFFICE

2,143,352

## PROCESS OF IMPROVING TEXTILE MATERIALS

Ernst Koch, Georg Schulz, and Alfred Eckelmann, Frankfort-on-the-Main, Germany, assignors to I. G. Farbenindustrie Aktiengesellschaft, Frankfort-on-the-Main, Germany

No Drawing. Application December 5, 1935, Serial No. 53,005. In Germany December 13, 1934

10 Claims.

(Cl. 91—70)

The present invention relates to improved textile materials and to a process of producing same.

In the copending application Ser. No. 739,714 of Josef Stadler there is described a process of rendering textile materials substantially resistant to creasing, which comprises impregnating the said materials with an aqueous solution of a compound reacting as formaldehyde in the presence of a non-oxidizing acid-reacting compound, acting on the said material with an organic "non-resin compound" containing a basic group and at least one radicle with at least four carbon atoms and heating to an elevated temperature.

15 We have now found that textile materials may also be improved without the addition of acid or compounds having an acid reaction by treating them with salts of amines having more than five carbon atoms in the molecule and an aldehyde and subjecting the textile materials to a treatment at elevated temperatures. Salts suitable for the said process are for example the chlorides, sulphates and oxalates of those amines which contain a cyclic or heterocyclic radicle or 20 a straight or branched carbon chain with more than five carbon atoms, which chain may also be interrupted by other atoms or atomic groups, such as oxygen or sulphur atoms or  $=NH$  groups. Particularly suitable are soluble salts of the said 25 amines. Salts of the said kind are for example octylamine hydrochloride, dodecylamine sulphate, stearylamine acetate, the hydrochlorides, sulphates, formates, lactates or oxalates of amines obtained from commercial stearic acid, 30 coconut fatty acids, palm kernel oil fatty acids, train oil fatty acids, naphthenic acids, montanic acids or resinic acids, for example by converting the said acids into their nitriles and reducing the nitriles. Octylfurfurylamine hydrochloride, 35 glucamine sulphate and phenylstearylamine hydrochloride may also be employed as initial materials. The presence of larger amounts of acids than are necessary for the formation of salts of the said amines is to be avoided in the present 40 case. The said salts may be employed in the form of their solutions or dispersions.

45 As aldehydes may be used in the present process for example formaldehyde, acetaldehyde, glyoxal and the like. Particularly suitable are the 50 aliphatic aldehydes having a low molecular weight. The aldehydes may be employed in the form of their aqueous solutions, or for example in the case of formaldehyde, also in the gaseous state.

55 The impregnated textile materials are subse-

quently treated at temperatures above 100° C.; preferably temperatures of from about 100° to 200° C., are employed. Generally speaking it is sufficient to heat the textile materials for a short time for example for 15 to 60 minutes up to 5 about 100° to 120° C.

The textile fibres or fabrics treated according to the process described possess a good stability to creasing and an agreeable soft touch.

The following examples serve to illustrate how 10 the present invention is carried out in practice, but the invention is not restricted to these examples. The parts are by weight.

## Example 1

15

20 parts of dodecylamine hydrochloride are dissolved in 200 parts of warm water and then 300 parts of a 35 per cent solution of formaldehyde are added. In this solution viscose artificial silk fabric is handled for 15 minutes at room temperature, then squeezed off and dried at about 50° C. The fabric is then treated for a short time at from about 100° to 110° C. on the tension frame or a cylindrical drier.

## Example 2

25

30 parts of stearylamine sulphate and 30 parts of commercial glyoxal are dissolved in 300 parts of distilled water. A viscose artificial silk fabric is impregnated by handling it for a short time 30 at room temperature in this solution and then treated at about 100° C. The fabric thus treated becomes very stable to creasing.

## Example 3

35

8 parts of the hydrochloride of the commercial mixture of amines (obtainable by converting coconut fatty acids into their nitriles and reduction of the said nitriles) are dissolved in 100 parts of water. In this solution viscose artificial 40 silk fabric is treated for about 10 minutes at between 15° and 20° C., squeezed off and then treated for about 20 minutes in a space containing formaldehyde vapors. The fabric is then subjected to a heat treatment as described in Example 1. It has become stable to creasing and 45 has a soft touch.

What we claim is:

1. The process of rendering textile materials 50 resistant to creasing which comprises causing a salt of an aliphatic amine containing more than five carbon atoms in the molecule and an aldehyde to act on textile materials and heating the textile materials to an elevated temperature.
2. The process of rendering textile materials 55 resistant to creasing which comprises causing a

- salt of an aliphatic amine containing more than five carbon atoms in the molecule and an aldehyde to act on textile materials and heating the textile materials to a temperature from about 5 100° to about 200° C.
3. The process of rendering textile materials resistant to creasing which comprises causing a salt of an aliphatic amine containing more than five carbon atoms in the molecule and an aldehyde to act on textile materials and heating the textile materials to a temperature from about 10 100° to about 120° C.
4. The process of rendering textile materials resistant to creasing which comprises causing a salt of an aliphatic amine containing more than 15 five carbon atoms in the molecule and an aldehyde to act on textile materials in an aqueous medium and heating the textile materials to an elevated temperature.
5. The process of rendering textile materials 20 resistant to creasing which comprises causing a water-soluble salt of an aliphatic amine containing more than five carbon atoms in the molecule and an aldehyde to act on textile materials and heating the textile materials to an elevated temperature.
6. The process of rendering textile materials 25 resistant to creasing which comprises causing a water-soluble salt of an aliphatic amine containing at least one carbon chain with from 8 to 18 carbon atoms and formaldehyde to act on textile materials and heating the textile materials to an elevated temperature.

7. The process of rendering textile materials 5 resistant to creasing which comprises causing a water-soluble salt of an aliphatic amine containing at least one carbon chain with from 8 to 18 carbon atoms and glyoxal to act on textile materials and heating the textile material to an elevated temperature.

8. The process of rendering textile materials 10 resistant to creasing which comprises causing a mixture of water-soluble salts of aliphatic amines derived from fatty acids of vegetal origin and a low molecular aliphatic aldehyde to act on textile materials and heating the impregnated materials to an elevated temperature.

9. The process of rendering textile materials 15 resistant to creasing which comprises causing a salt of an aliphatic amine containing more than five carbon atoms in the molecule and an aldehyde in gaseous state to act on textile materials and heating the textile materials to an elevated 20 temperature.

10. The process of rendering textile materials 25 resistant to creasing which comprises causing a salt of an aliphatic amine containing more than five carbon atoms in the molecule and an aldehyde in gaseous state to act on textile materials and simultaneously heating the textile materials to an elevated temperature.

ERNST KOCH. 30  
GEORG SCHULZ.  
ALFRED ECKELMANN.